

Dec. 8, 1964

J. R. A. BEALE ET AL

3,160,799

HIGH-FREQUENCY TRANSISTOR

Filed Dec. 8, 1960

2 Sheets-Sheet 1



FIG.1



FIG.2

INVENTOR  
JULIAN R. A. BEALE  
ANDREW F. BEER  
BY  
*Frank R. Sinfani*  
AGENT

Dec. 8, 1964

J. R. A. BEALE ET AL

3,160,799

HIGH-FREQUENCY TRANSISTOR

Filed Dec. 8, 1960

2 Sheets-Sheet 2



FIG. 3



FIG. 4



FIG. 5



FIG. 6



FIG. 7

INVENTOR  
JULIAN R. A. BEALE  
ANDREW F. BEER

BY  
Frank R. Jinfari  
AGENT

# United States Patent Office

3,160,799

Patented Dec. 8, 1964

1

3,160,799

## HIGH-FREQUENCY TRANSISTOR

Julian Robert Anthony Beale, Reigate, and Andrew Francis Beer, Downside, Epsom, England, assignors to North American Philips Company, Inc., New York, N.Y., a corporation of Delaware

Filed Dec. 8, 1960, Ser. No. 74,544

Claims priority, application Great Britain Dec. 14, 1959  
4 Claims. (Cl. 317—235)

The invention relates to a transistor comprising a semi-conductive body, to which an emitter electrode and a base electrode are applied side by side in the form of alloy electrodes, of which the associated zones of recrystallized semi-conductive material establish a contact with the base zone, and furthermore to a method of manufacturing such a transistor. The term "alloy electrode" on a semi-conductive body is to be understood to denote herein an electrode obtained by causing a quantity of electrode material to be alloyed in a molten state on the surface of the semi-conductive body below the melting point of the semi-conductive material of this body to dissolve an adjacent part of the semi-conductive body and subsequently, by cooling, causing firstly part of the dissolved semi-conductive material to recrystallize in the form of a zone grown on the semi-conductive body, the so-called recrystallized zone, after which the remainder of the melt solidifies, which consists for the major part of the alloyed electrode material, termed hereinafter the solidified zone. This solidified zone is separated by the recrystallized zone from the initial material of the body. The semi-conductive material of the recrystallized zone may have absorbed active impurities from the alloyed material, these impurities determining its specific conductivity and its conductivity type. In the present case the recrystallized zone of the emitter is of a conductivity type opposite that of the base zone and the recrystallized zone of the base electrode has a conductivity type equal to that of the base zone.

The base zone may, for example, be formed by the semi-conductive body itself. In order to enlarge the frequency range of the transistor towards the higher frequencies, attempts were made to minimize the distance between the base electrode and the emitter and, moreover, the thickness of the base zone. It is known to obtain by a diffusion method with a suitable active impurity such a thin base zone of which the conductivity type is opposite that of the remainder of the semi-conductive body, constituting in this case the collector zone. Such a base zone obtained by a diffusion method may be provided as a whole prior to the provision of the emitter electrode and the base electrode. It may be formed also, at least partly, during the provision of at least one of these alloy electrodes by diffusion of a rapidly diffusing impurity out of the alloyed electrodes into the adjacent semi-conductive material. At the same time an impurity may be introduced by diffusion out of the ambient atmosphere into the surface of the semi-conductive body adjacent the electrode. This impurity may, for example, be evaporated from the electrode material itself.

The invention has for its object inter alia to enlarge further the frequency range of a transistor comprising a semi-conductive body to which the emitter electrode and the base electrode are applied side by side in the form of alloy electrodes, of which the associated zones of recrystallized, semi-conductive material establish a contact with the base zone. In accordance with the invention, the transistor is characterized in that the recrystallized material of at least one of these electrodes is removed from the side remote from the other electrode over at least half of the contact surface initially occupied by the recrystallized zone with the base zone. In

2

this manner, for example, the internal capacitances harmful to a high-frequency range may be reduced without involving an increase in distance between the emitter electrode and the base electrode. In this case recrystallized material may have been removed only from the base electrode. Recrystallized material is, however, preferably removed at least from the emitter, so that the capacitance of the rectifying emitter-base junction is reduced. The contact surface between the recrystallized zone and the base zone is preferably not more than one quarter of the initial contact surface.

It should be noted that it is known per se with a transistor having a base zone formed by diffusion, on which are provided an emitter electrode and a base electrode closely to each other, to remove the base zone beyond the parts covered by the two said electrodes and the part lying in between by etching as far as possible, so that the junction between the base zone and the collector zone is reduced to a small surface, in order to reduce the capacitance of this junction. With such an etching process it is often unavoidable that a small part of the recrystallized zone of the emitter electrode and/or the base electrode is removed. However, the removal of recrystallized material over only a small part of the contact surface initially occupied by the recrystallized zone with the base zone is concerned there, whereas in the method according to the invention the recrystallized material is removed over at least half of the contact surface initially occupied by the recrystallized zone. The solidified zone which may then extend beyond the recrystallized zone, may still be sufficiently large for a satisfactory connection.

The removed material is preferably replaced by an insulating material, for example an insulating lacquer. Thus the projecting part of the solidified zone can be adequately supported.

This distance between the emitter electrode and the base electrode is preferably small, for example smaller than ten-thousandths of an inch. The dimensions of the surface occupied by the recrystallized zone may then be of the same order of magnitude, whereas the dimensions of the solidified zone may be much larger.

Underneath at least part of the initial contact surface, where the recrystallized material has been removed, the base zone itself is preferably also removed, so that also the contact surface between the collector zone and the base zone and hence the capacitance between the base and the collector are further reduced.

The invention furthermore relates to a method of producing a transistor comprising a semi-conductive body, to which the emitter electrode and the base electrode are applied side by side in the form of alloy electrodes, of which the associated zones of recrystallized, semi-conductive material establish a contact with the base zone. According to the invention this method is characterized in that subsequent to the application of these alloy electrodes the part of the surface of the semi-conductive body between these electrodes is covered by a material insensitive to etching agents, after which the assembly is subjected to etching, so that the recrystallized material of at least one of these two electrodes is removed from the side remote from the other electrode over at least half of the contact surface with the base zone occupied by the recrystallized zone.

The etching process is preferably carried out until at the most one quarter of the contact surface occupied by the recrystallized zone with the base zone remains.

The etching process is preferably carried out in several stages with intermediate measurement of the capacity of the base-emitter junction. More than one etching bath may be used, preferably with etching agents of different concentrations and/or by using different current

passages, so that in the first stage the etching process is performed more rapidly than during the subsequent stages, in order to obtain the desired capacity more accurately. This method is quite suitable for automation methods, for example, by interrupting the etching process by means of a servo-mechanism automatically when the desired capacity is attained or has dropped just below the desired value.

After the application of the alloy electrodes and prior to the etching process of at least one of the alloy electrodes, one part may be removed mechanically, for example by cutting, from the side remote from the other electrode. In this manner the final shape of the remaining recrystallized zone, subsequent to etching, depends less upon the initial shape of the alloy electrode, so that the final shape is better controllable by choosing a suitable shape of the front from where etching starts.

Embodiments of the method and the transistor according to the present invention will now be described, by way of example, with reference to the accompanying diagrammatic drawing, in which:

FIGURE 1 is a cross-sectional view of part of a transistor.

FIGURE 2 is a plan view of part of the transistor shown in FIGURE 1.

FIGURE 3 shows a test circuit for measuring the capacity between emitter and base.

FIGURE 4 is a block schematic representation of an etching procedure in several steps in the method according to the present invention.

FIGURES 5 and 6 are partial plan views of two further transistors and

FIGURE 7 is a partial cross-sectional view of the transistor shown in FIGURE 6.

In the figures section shading has been omitted for the sake of clarity and the same reference numerals are used to indicate similar components or features.

Referring now to FIGURES 1 and 2, a transistor comprises a resolidified region 1 consisting mainly of lead with about 1% by weight of antimony and including a little germanium, an n-type germanium region 2 consisting mainly of germanium and including a little lead and a little antimony, a resolidified region 3 consisting mainly of lead, antimony and aluminum and including a little germanium, a recrystallized p-type germanium region 4 consisting mainly of germanium and including a little lead, antimony and aluminum, an n-type base region 5 consisting mainly of germanium into which antimony has been diffused, an unchanged part 6 of an originally rectangular single crystal slice of p-type germanium of dimensions originally about 2 mms. x 2 mms. x 6-thousandths of an inch and having a resistivity of 2 ohm-cm., constituting the collector zone, a recrystallized p-type region 7 consisting mainly of germanium and including a little indium and gallium and a resolidified region 8 consisting mainly of indium and gallium and including a little germanium. The different semiconductive regions are only designated schematically in FIGURE 1. For instance in reality the recrystallized zones 2 and 4 will extend only very slightly beyond the respective resolidified regions 1 and 3. Fine nickel wires 9 and 10 and a stout nickel wire 11 are soldered to the regions 1, 3 and 8 with the use of indium solder 16, 17 and 15, respectively. The wire 9 forms a connection to the base, the wire 10 forms a connection to the emitter and the wire 11 forms a connection to the collector of the transistor and in addition is used as a mechanical support.

The region 1 and the region 2 are separated from the region 3 and the region 4 by a slot 12 which is about 1-thousandth of an inch wide at its bottom. The slot 12 is filled to the level indicated by the broken line 13 with polystyrene lacquer applied as a solution in ethylmethylketone.

The transistor as described above may be made in the following way.

On the originally rectangular single crystal slice of p-type germanium a pellet in the shape of a circular disc about two-thousandths of an inch thick and eight-thousandths of an inch in diameter, consisting of lead with 1% by weight of antimony, is applied and an alloy contact is made by heating the whole to about 700° C. for about 3 minutes in an atmosphere of hydrogen. After cooling the slot 12 is applied penetrating the alloy contact and its recrystallized region and extending slightly into the undissolved p-type material of the body. This slot divides the alloy contact into two parts. The slot may be manufactured by ultrasonic cutting using a thin cutting head and a slurry of a fine abrasive, e.g., aluminum oxide abrasive.

Some aluminum is applied to only one part of the alloy contact and the whole is then heated in an atmosphere of hydrogen for about 10 minutes at 750° C. during which the two parts of the contact are molten and antimony diffuses from the two molten parts into the material of the body underneath the molten parts and into the adjacent surface parts of the body including the bottom part of the slot 12, thus forming the n-type region 5. By cooling the two recrystallized regions 2 and 4 and the resolidified regions 1 and 3 are formed. The p-type region 7 and the resolidified region 8 may be made in a manner known per se by melting a pellet, consisting of an indium-gallium alloy, onto the germanium body.

The transistor described above is now immersed in an electrolytic etching bath containing an aqueous solution of sodium hydroxide, e.g., a 5% solution. The three wires 9, 10 and 11 are connected to the positive terminal of a voltage source and a platinum electrode in the bath is connected to the negative terminal of the voltage source. A large amount of the recrystallized material 2, 4 and 7 is etched away from beneath the resolidified regions 1, 3 and 8, so that the area of contact between the recrystallized material 2 and 4 and the n-type region 5 is reduced to be not more than one half of the area of contact present after alloying and before etching. The resolidified regions 1 and 3 are not attacked substantially by the etching medium and thus undercutting of the regions 1 and 3 occurs.

The broken lines 18, 19 and 20 show three intermediate stages during the etching step, the final stage being indicated by the line 20a. The etching may be continued until the areas of contact between the regions 2 and 4 and the regions 1 and 3 are not more than one quarter of the area of contact before the etching step. In a typical case, the initial dimension *a* is 9 thousandths of an inch and the dimension *b* at the end of the prolonged etching step about 4 thousandths of an inch (see FIGURE 1). The areas of contact between the regions 1 and 3 and the region 5 are reduced to about the same extent.

After this etching step, the polystyrene lacquer in the slot is removed using ethylmethylketone as a solvent, and the whole is immersed in an etching bath for a final etch in 20 volumes hydrogen peroxide at 70° C. for about 15 seconds. The regions 1, 3 and 5 are then covered with a mass 14 of polystyrene lacquer dissolved in ethylmethylketone, the lacquer penetrating into the gaps below the regions 1 and 3 and giving mechanical strength to the transistor.

FIGURE 2 shows only the slot 12 and the lines 18, 19, 20 and 20a which are substantially circular in form since the outer contour of the regions 1 and 3 joined together by the lacquer provided in the slot 12 before the prolonged etching step is initially substantially circular.

The transistor so produced is then encapsulated in any known manner.

The transistor described above has low emitter-base and base-collector capacitances due to the severe reduction of the area of the base-emitter junction and the base-collector junction.

The extent to which the etching is effected may be controlled by monitoring the capacitance of the base-emitter junction which has low-resistivity material at each side. The capacitance is sufficiently high to measure even if the junction area is small. FIGURE 3 shows a test circuit for measuring the base-emitter junction capacitance. The test circuit comprises a generator 21 of signals having a frequency of about 20 mc./s. at a small signal strength of about 50 mv. (R.M.S.). The generator 21 is connected in series with the emitter-base junction of the transistor and a resistor 22, conductor 23 being connected to the transistor emitter and conductor 24 being connected to the transistor base. The signal developed across resistor 22 is measured by means of a vacuum tube volt-meter 25 and gives an indication of the base-emitter junction capacitance.

It is found that this capacitance can be measured even if the transistor is immersed in water if care is taken that the resistivity of the water is high, for example, is greater than 1,000 ohm-cms. There will be stray capacitance due to the connections to the base and the emitter and this is increased if the transistor is immersed in water which has a dielectric constant of approximately 80. It is, however, found that the base-emitter junction capacitance at zero bias can be monitored in this way down to a value of about 7 pf., the stray capacitance with the transistor immersed in water being about  $3 \pm 1$  pf.

FIGURE 4 is a schematic diagram showing an apparatus in which the prolonged etching step may be carried out. A number of stations are provided etching being carried out at alternate stations 26 and washing in water and testing being carried out at the other alternate stations 27. Testing is carried out by a circuit as described above with reference to FIGURE 3, the voltage developed across the resistor 22 during testing being supplied not to a volt-meter but to a control device determining whether further etching is necessary. The apparatus also comprises a loading station 28 and an unloading station 29. A transistor is inserted in a holder at station 28 and is thereafter moved to the first etching station 26 where the transistor is automatically connected for etching and is immersed in etching fluid in a bath 30. After a predetermined time, the transistor is moved to the first testing station 27, is connected to the conductors 23 and 24 of the test circuit and is immersed in a bath 31 of washing water. When washing has been effected for a sufficient time, the test circuit 32 is switched on and the base-emitter junction capacitance is measured. If the capacitance has not been sufficiently reduced, the transistor is moved to the second etching station 26 along a path indicated by the broken line 33 and is again subjected to etching with the use of a bath 30 after which it is moved to the second testing station 27. Similar procedures are followed at each succeeding station 26 and 27 until the desired capacitance is reached. When the desired capacitance is reached, the output of the test circuit 32 causes operation of a relay device 34 so that no further etching is effected. The broken line 33 indicates the path of the device. The transistor finally reaches the unloading station 29 where it is removed from the apparatus. It is not necessary to etch to the same extent at each of the stations 26, it may be preferred to etch to a considerable extent at the first station 26 and thereafter to etch more lightly at the succeeding stations 26 in order gradually to reach the desired capacitance. Further the extent of etching at a subsequent station may be made dependent on the capacitance measured at the preceding test.

The apparatus is shown in the schematic drawing of FIGURE 4 arranged in a linear manner, but it will be obvious that the apparatus may be a rotary apparatus and further that a single testing circuit may be used and connected in turn to each station 27 for testing before the line of transistors moves on to the succeeding stations so that unloading and reloading in turn of the holders for the transistors may be effected.

The etching procedure may also be applied to a transistor comprising two alloy zones provided by alloying at two separate areas of a semi-conductor body, as indicated in FIGURE 5. It is remarked that in general the two zones may be separated by as little as two thousandths of an inch and the dimension of each zone in the direction of separation of the zones may be about 8-thousandths of an inch.

The transistor comprises two resolidified regions 36 and 37. The regions 36 and 37 are connected to wires (not shown) by solder (not shown). A region 38 of an etch-resistant material is provided between the two regions 36 and 37, for example, applied with a paint-brush. The transistor is then etched in the manner described with reference to FIGURES 1 and 2, progressive stages of etching being indicated by the broken lines 39.

An alternative method is illustrated in FIGURES 6 and 7. Before the wires (not shown) are secured in position, a portion of each resolidified region 36 and 37 remote from the other resolidified region is removed and in the transistor illustrated about half of each, the shaded portions 40 and 41, are removed, for example, with a sharp blade. The wires (not shown) are connected and the etch resistant region 38 provided and subsequent progressive stages of etching are indicated by the lines 39, the full line 39 in FIGURE 7 indicating the final extent of etching. It will be noted that in this case no thin elongated area of contact between the recrystallized material and the resolidified produced as shown in FIGURE 5 is obtained, but a short broader area of contact as indicated in FIGURES 6 and 7, by which a lower base resistance is obtained in this latter embodiment.

It will be noted that for all three embodiments, those of FIGURES 1 and 2, FIGURE 5 and FIGURES 6 and 7, the size of the resolidified regions are greater than the areas of contact between the recrystallized material and the base region remaining after etching and hence that for a given remaining area of contact it is, in each case, comparatively simple to attach wires to the resolidified regions.

As an alternative to the use of polystyrene lacquer and ethylmethylketone as a solvent, other etch-resistant lacquers and other solvents may be used, e.g., Cerric Black Resist available commercially under the reference DH 5353 from Cellon Limited may be used and acetone as a solvent.

What is claimed is:

1. A high-frequency transistor comprising a semiconductive body having a collector region of one conductivity type and a thin diffused base region of the opposite conductivity type, and separate emitter and base electrodes alloyed adjacent to one another on the same surface of the body forming emitter and base recrystallized regions, respectively, contacting the base region, said base recrystallized region being of the same type conductivity as that of the base region, said emitter recrystallized region being of the opposite type conductivity to that of the base region, the semiconductive body portions underneath the emitter electrode and on the side thereof remote from the base electrode being cut away such that the cross-sectional area in a plane parallel to the body of at least the emitter recrystallized region is at most one-quarter the corresponding cross-sectional area of the overlying emitter electrode and the latter has at least three-quarters of its area on the side remote from the other electrode extending over and free of direct contact with the semiconductive body, said emitter and base electrodes being spaced apart a distance less than 0.010 inch, the size of said emitter and base electrodes in the direction of their separation being no greater than 0.040 inch.
2. A transistor as set forth in claim 1 wherein insulating material is disposed between the semiconductive body and the electrode portion extending over and free of direct contact with the said body.
3. A transistor as set forth in claim 1 wherein the size

of each of the emitter and base electrodes in the direction of their separation is no greater than the distance of their separation multiplied by a factor of four.

4. A high-frequency transistor comprising a semiconductive body having a collector region of one conductivity type and a thin diffused base region of the opposite conductivity type, separate emitter and base electrodes alloyed adjacent to one another on the same surface of the body forming emitter and base recrystallized regions, respectively, contacting the base region, said base recrystallized region being of the same type conductivity as that of the base region, said emitter recrystallized region being of the opposite type conductivity to that of the base region, the semiconductive body portions underneath each of the emitter and base electrodes on the side of each remote from the other being cut away such that the cross-sectional area in a plane parallel to the body of each of the recrystallized regions is no greater than one-quarter the cross-sectional area of their overlying electrodes and the latter have at least three-quarters of their area on the side remote from the other electrode extending over and free of direct contact with the semiconductive body, said

emitter and base electrodes being spaced apart a distance less than 0.010 inch, the size of each of said emitter and base electrodes in the direction of their separation being no greater than the distance of their separation multiplied by a factor of four.

References Cited in the file of this patent

UNITED STATES PATENTS

|           |                   |               |
|-----------|-------------------|---------------|
| 2,829,422 | Fuller            | Apr. 8, 1958  |
| 2,842,831 | Pfann             | July 15, 1958 |
| 2,876,401 | Fuller            | Mar. 3, 1959  |
| 2,956,217 | Meyerhofer        | Oct. 11, 1960 |
| 2,980,983 | Beale et al.      | Apr. 25, 1961 |
| 3,069,297 | Beale             | Dec. 18, 1962 |
| 3,081,418 | Manintveld et al. | Mar. 12, 1963 |

FOREIGN PATENTS

|         |               |                |
|---------|---------------|----------------|
| 849,477 | Great Britain | Sept. 28, 1960 |
|---------|---------------|----------------|

OTHER REFERENCES

Shive: Semiconductor Devices, D. Van Nostrand Co., Inc., 1959, pages 76 and 97.